

M. M. MERRITT.  
ELECTROLYTIC PROCESS.  
APPLICATION FILED JUNE 27, 1917.

1,282,264.

Patented Oct. 22, 1918.

Fig. 1.



Fig. 2.



INVENTOR:  
Matthew M. Merritt,  
By Emma Northway, Name  
Attest.

# UNITED STATES PATENT OFFICE.

MATTHEW M. MERRITT, OF DANVERS, MASSACHUSETTS, ASSIGNOR TO COPPER PRODUCTS COMPANY, OF BOSTON, MASSACHUSETTS, A CORPORATION OF MAINE.

## ELECTROLYTIC PROCESS.

1,282,264.

Specification of Letters Patent.

Patented Oct. 22, 1918.

Application filed June 27, 1917. Serial No. 177,173.

To all whom it may concern:

Be it known that I, MATTHEW M. MERRITT, a citizen of the United States, and a resident of Danvers, county of Essex, Commonwealth of Massachusetts, (whose post-office address is Danvers, Massachusetts), have invented an Improvement in Electrolytic Processes (A), of which the following description, in connection with the accompanying drawings, is 10 a specification, like characters on the drawings representing like parts.

This invention pertains to improvements in electrolytic processes, and more particularly, though not exclusively, to improvements in depositing copper or other metal on the surface of cylindrical or other mandrels, and of separating the deposited sheets from the mandrel to form continuous sheets, while reducing to a minimum that portion of 20 the sheet which must be cut away to provide smooth edges therefor.

In the drawings, which show one illustrated embodiment of a preferred form of electrolytic apparatus well suited for use in 25 connection with my novel process;

Figure 1 is a section through an electrolytic bath, showing in elevation a rotatable cylindrical drum which is to serve as a cathode for the electrolytic deposit of the 30 copper or other metallic sheet;

Fig. 2 is a diagrammatic section through a portion of the drum.

In the drawings I have shown a rotatable cylindrical drum 1 partially immersed in an 35 electrolytic bath 2, the surface of the drum serving as a cathode for the deposit of a sheet 4 of copper or other metal which is adapted to be stripped from the surface of the drum preferably in the form of a helix, 40 so that using a drum of a given circumference, a sheet of copper or other metal of much greater length may be formed thereon. In the preferred form of my invention, I prefer to apply the current to produce a

45 slight film 6 of electrolytic deposit over the surface of the mandrel which has been previously treated with any suitable preparation 7 for preventing the permanent adhesion of the deposit to the mandrel. After 50 a small amount of copper has been deposited upon the entire surface of the mandrel, I apply on the surface of such copper deposit a non-conductive flexible element preferably forming a helix about the drum. This flexible element may take the form of the piece

of string 5 coated with shellac, or a wire coated with any suitable insulating substance. I then again apply power to rotate the drum, and again apply the current to continue the electrolytic deposit until the 60 deposited sheet is of the required thickness.

The copper may then be stripped from the mandrel, and I find that it will tear very readily along the lines of the flexible non-conductive element. It is not essential that a 65 preliminary electrolytic deposit be made prior to the application of the flexible non-conductive element which forms the helix, but the use of the preliminary deposit is preferable because this protects the surface of 70 the mandrel from the flexible element, and prevents any disturbance of the preliminary coating thereon, while, where plastics such as shellac are used on the flexible element, it prevents the deposit of such plastic on the 75 mandrel, which would cause irregularities in metallic sheets subsequently formed thereon. In such case the deposit of such plastic is in the metallic sheet itself, and all irregularities are confined to a very narrow strip of metallic deposit. This permits the reduction to a minimum of the edges of the sheet which need be trimmed, and under some conditions renders trimming entirely 80 unnecessary.

The details of the bath, the construction of the drum and its operation, other than above described, form no part of the present invention, but are described and claimed in copending applications filed herewith. 85

While I have illustrated one form of apparatus, and while I have described one specific embodiment of my novel process in connection with the described apparatus, it will be understood that changes in the apparatus and in the specific processes herein described may be made within the scope of the appended claims. 90

### Claims:

1. The process of forming metallic sheets, 100 which comprises electrolytically depositing a thin sheet of metal upon a mandrel, winding a non-conductive flexible element about said mandrel, continuing the electrolytic deposit, and removing the thickened sheet 105 from said mandrel by tearing said sheet along the line defined by said flexible non-conductive element.

2. The process of forming a metallic sheet, 110 which comprises electrolytically depositing

- a thin sheet of metal upon a rotating partially submerged mandrel, winding a non-conductive flexible element in a helix about said mandrel above said thin sheet, continuing the electrolytic deposit while rotating said mandrel until said sheet is increased in thickness to the desired extent, and removing said sheet from said mandrel by tearing along the line of the helix defined by said non-conductive flexible element.
3. The process of dividing galvanoplastic deposits formed on a rotating cathode,

which comprises electrolytically depositing a thin sheet of metal upon the surface of the cathode, locating a non-conductive element on said thin sheet along a proposed line of division, continuing the electrolytic deposit until said thin sheet has been increased in thickness to the desired extent, and then tearing said sheet along a line defined by said non-conductive element. <sup>15</sup>

In testimony whereof I have signed my name to this specification.

MATTHEW M. MERRITT.